

# United States Patent Office.

HENRY A. PEASE, OF HARTFORD, CONNECTICUT.

*Letters Patent No. 99,468, dated February 1, 1870; antedated January 21, 1870.*

## IMPROVEMENT IN THE MANUFACTURE OF SOAP.

The Schedule referred to in these Letters Patent and making part of the same.

*To all whom it may concern:*

Be it known that I, HENRY A. PEASE, of Hartford, county of Hartford, and State of Connecticut, have invented a new and useful Improvement in the Manufacture of Soap; and I declare the following to be a full and exact description thereof.

My improvement relates to the manufacture of hard soap, as contradistinguished from soft or liquid soap.

The process is as follows:

Take, say, seventy-five (75) pounds of tallow, stearine, or lard-oil, pour it into a kettle, and heat to about one hundred (100) degrees centigrade; a variation of a degree or two will do no hurt. Add one (1) pound of borax, skim off the scum which soon rises, and allow to cool. When cooled to about ninety (90) degrees, (centigrade always,) having provided one hundred and thirty-five (135) pounds of caustic soda-lye, of twenty-one (21) degrees' strength, add the lye slowly, till the mixture thickens. Care must be taken to have the lye cold, and of the right strength. When the lye is all in, stir rapidly till all the constituents are thoroughly mingled. When this is done, having provided twenty-five (25) pounds of cocoa or other heavy vegetable oil, add the cocoa or other oil, which will tend to neutralize the lye. When the mixture becomes free from a sharp bite, when applied to the tongue, then heat until the whole is transparent, glossy, and without spots. Now put it, expeditiously, into moulds or forms, and allow to harden.

Having proceeded thus far, I have produced a soap which is perfect, in its way, and which is vendible; but as I still further refine the soap, and produce a still finer article, I will, for convenience' sake, designate the process already described, as the "preliminary process," and the soap already produced, as the "preliminary product."

I will now describe how I further refine my soap.

Take the "preliminary product," when it is cold and hard, and reduce it to powder. Put the powder into

a kettle and heat slowly. For every pound of powder, provide one (1) pint of gin, or other spirituous liquor, (preferably gin,) and commence putting into the kettle, after the powder is in, beating up the mixture as you pour, for it will froth. As soon as the powder melts or liquefies, it will at once become solid. Add the gin or other liquor gradually, with care, for the mixture will rise in the kettle. The mixture will soon gloss over on the surface. Continue to add the liquor till all in. Then heat till the whole forms a beautiful, transparent, jelly-like mass. Now, add to every twenty (20) pounds of soap, seven (7) ounces of some perfuming-essence, or its equivalent of essential oil, for perfumery, and stir till thoroughly mixed. Then put into form expeditiously, stir till it begins to harden, and then cover up.

The product, designated herein as the "final product," produced by this last process, called herein the "final process," is an excellent article for the toilet or medical uses.

I claim, as my invention—

1. The combination of ingredients described, forming the composition designated herein as the "preliminary product," the same being compounded together by the process described herein as the "preliminary process."

2. As an article of manufacture, the compound designated herein as the "preliminary product."

3. The combination of ingredients, described herein, forming the compound designated herein as the "final product," the same being compounded together by the process described herein as the "final process."

4. As an article of manufacture, the compound described herein as the "final product."

Dated May 21, 1869.

HENRY A. PEASE.

Witnesses:

W. E. SIMONDS,  
WM. W. HYDE.